

# UNITED STATES PATENT OFFICE.

WILLIAM A. BOLE, OF PITTSBURGH, PENNSYLVANIA.

## METHOD OF MAKING CASTINGS.

1,227,573.

Specification of Letters Patent. Patented May 29, 1917.

No Drawing. Application filed September 25, 1912, Serial No. 722,218. Renewed April 12, 1917. Serial No. 161,671.

To all whom it may concern:

Be it known that I, WILLIAM A. BOLE, a citizen of the United States, and a resident of Pittsburgh, in the county of Allegheny 5 and State of Pennsylvania, have made a new and useful Invention in Methods of Making Castings, of which the following is a specification.

This invention relates to improvements in 10 the art of metal-casting.

It has been known for some time that the 15 defects in cast metal, particularly cast iron and steel, are in a large measure due to the absorption of oxygen by the molten metal while in the mold or while entering the mold, and that this to a great extent could be remedied by filling the mold with an inert 20 gas such as carbon dioxide (CO<sub>2</sub>). By filling the mold with an inert gas before the metal is poured into the same, air with its contained oxygen is expelled and 25 castings free from defects due to the absorption of oxygen can be produced. As the amount of inert gas necessary,—especially where large castings or ingots are made,—must be large, the methods heretofore suggested or utilized, so far as I am aware, have been unsuccessful, principally due, I believe, to the cost of the gas employed.

30 My invention consists in employing for the purpose of filling the mold, which may either be a sand mold as in ordinary cases of iron or other metal-casting, or metal molds as employed in making ingots, gases whose 35 cost is low, such as the exhaust gases from an internal combustion engine or flue gases which are the products of combustion. I have found by experience that either of these gases; that is, the exhaust gases from an internal 40 combustion engine or flue gases, are sufficiently devoid of oxygen for this use, and that by using them I obtain a cheap method of preventing the defects in castings or ingots due to the absorption of oxygen 45 while the molten metal is in the mold, or while entering the mold.

If desired, the exhaust gases from internal combustion engines or flue gases may be

scrubbed and dried, or otherwise cleaned and stored for use, and then conveyed 50 into the molds from which the atmospheric air is to be expelled and excluded, or the gases may be led directly from their source to the molds. The gases for filling the molds may either be led into the molds from 55 the bottom or spilled into them from the top.

If desired, a retainer for the inert gas may be used which projects above the top 60 of the mold so that the molten metal will be poured into the mold through an inert atmosphere and in fact the entire distance from the source of molten metal to the mold may be made to consist of inert gas when cheap gas, such as my invention contem- 65 plates, is used.

Having thus described my invention, what I claim is:

1. The method of preventing the absorption of oxygen by molten metal during the 70 operation of casting the metal, which consists in filling the mold space with an excess of relatively heavy dry gaseous products of combustion, in submerging the pouring hole of the mold with dry gaseous products of 75 combustion, and then pouring the molten metal to be cast through the gaseous atmosphere above the mold and into the mold.

2. The method of preventing absorption 80 of oxygen during the operation of casting, which consists in filling the mold with an excess of inert dry gaseous products of combustion in such quantities that the pouring hole communicating with the upper end of the mold is maintained submerged by the 85 inert gas, and then in pouring the metal to be cast into the mold through the pouring hole.

In testimony whereof, I have hereunto 90 subscribed my name this 20th day of September, 1912.

WILLIAM A. BOLE.

Witnesses:

Wm. P. FLINT,  
JOSEPH CONNELLY.